

1

3,400,121

**2,4,6-TRI-(1-AMINO-SUBSTITUTED AROMATIC)-s-TRIAZINES**

Gerhard Weckler and Siegfried Schiessler, Frankfurt am Main, Germany, assignors to Farbwerke Hoechst Aktiengesellschaft vormals Meister Lucius & Bruning, Frankfurt am Main, Germany, a corporation of Germany

No Drawing. Continuation-in-part of application Ser. No. 303,425, Aug. 20, 1963. This application Mar. 30, 1966, Ser. No. 538,609

3 Claims. (Cl. 260—239.7)

**ABSTRACT OF THE DISCLOSURE**

Novel compounds have been provided which are symmetrical 2,4,6-triazines of the formula:



in which A is lower alkylene, phenylene or naphthylene, Z is  $-\text{SO}_3\text{Y}$ ,  $-\text{OSO}_3\text{Y}$ ,  $-\text{COOY}$  or  $-\text{SO}_2\text{CH}_2\text{CH}_2\text{OSO}_3\text{Y}$

Y is hydrogen or a salt-forming cation, and n is an integer from 1 to 3, provided that when Z is  $-\text{SO}_3\text{Y}$  and  $-\text{COOY}$ , n is an integer from 2 to 3.

This application is a continuation-in-part of our application Ser. No. 303,425 filed Aug. 20, 1963 now U.S. Patent 3,278,253.

The present invention relates to improvements in the dyeing of textile materials such as yarns, filaments, fibers and fabrics having a basis of synthetic linear polyamides, as, for example, nylon. More particularly, the present invention relates to an improved process for dyeing yarns, filaments, fibers and fabrics made of, or essentially consisting of, synthetic linear polyamides with acid dyestuffs, complex metal dyestuffs or reactive dyestuffs or mixtures thereof.

It is well known in the art that textile materials made from polyamides can be dyed with various dyestuffs, for example, with acid wool dyestuffs, metal complex dyestuffs or chrome dyestuffs, at temperatures below and above 100° C. However, the dyeings thus produced are not satisfactory, because in most cases it is not possible to level irregularities of the yarn which are mainly caused by variations of the titer and differences in stretching and fixing. These yarn irregularities are distinctly visible after dyeing as streaks, bands or in the form of an unsettled appearance, depending on the type of goods, and they considerably reduce the sales value of the goods.

To by-pass these drawbacks, it has been proposed, in addition to selecting a suitable dyestuff, to retard the dyeing process and to carry it out in the presence of swelling agents in order to augment the penetration into the fiber, and thus to prevent blocking effects. As swelling agents, there have been used, for example, phenols and chlorinated, aromatic substances. These products, however, involve a number of disadvantages. They are, in most cases,

2

not simple to use and they are effective only in high concentrations. In addition, they are partly strongly absorbed by the fibers so that they can be removed later on with difficulty only and may then cause damage to the fibers. Although they reduce streakiness, they do not totally remove the streaks.

Furthermore, attempts have also been made to produce level dyeings through control of the substantivity of the dyestuff by shifting the pH-value of the dyebath during dyeing by the addition of a potentially acid dyeing assistant to the bath. However, this process does not remove or level streakiness of the fabric dyed.

Furthermore, it is known to use surface-active agents in the dyeing of polyamide fibers. Attempts have been made to produce level dyeings by adding cation-active dyeing assistants to the dyebath which are capable of forming complexes with acid wool dyestuffs, and to retard their penetration into the fiber. This process, too, does not yield satisfactory results, because the cation-active products tend to precipitate the acid dyestuffs. Even the addition of non-ionic dispersing agents to the dyebath does not remove the difficulties and does not offer the required reliability. Furthermore, there has been described the use of anion-active products which are added to the dyebath and which are to compete with the dyestuff for the free linking positions of the fibers. However, these products possess either such strong affinity for the polyamide fiber that all linking positions of the fiber are occupied by the dyeing assistant and that the dyebaths cannot be exhausted, or they are well able to retard the penetration of the acid dyestuff into the polyamide fiber in the case of light dyeings, but do not satisfactorily level out the streakiness.

Furthermore, products are described in the literature which are a combination of special, anion-active substances with complex-forming, weakly cation-active surface-active compounds such as polyvinyl pyrrolidone, or hydroxyethylated aminophenols.

In many cases these products are capable of levelling out the streakiness occurring with polyamide fibers when dyeing with acid dyestuffs; in the case of difficult dyeings with acid dyestuff combinations, they exhibit retarding effects which are different for each component of the dyestuff combination, so that dyestuff losses and alterations of shade are caused. The full effect of the mixtures is attained at temperatures above 100° C., so that anti-oxidizers must be used to prevent possible oxidations taking place at these high temperatures. In the dyeing of polyamide fibers with complex metal dyestuffs and reactive dyestuffs, fabric irregularities cannot be levelled out satisfactorily and a strong retardative effect is observed with some dyestuffs. A drawback is also the necessity of exactly adjusting the pH-value of the dyebath for obtaining optimum effects.

It is an object of this invention to provide an improved process for the more complete dyeing of textile materials having a basis of a synthetic linear polyamide with a dyestuff for said material. Another object of this invention is the provision of an aqueous dyebath comprising an acid dyestuff, a complex metal dyestuff, a reactive dyestuff or a mixture thereof and a particularly effective dyeing assistant. Other objects of this invention will be apparent from the following detailed description and claims:

We have found that streak-free dyeings on textile materials having a basis of a synthetic linear polyamide with

acid dyestuffs as well as with complex metal dyestuffs and reactive dyestuffs are obtained, when carrying out the dyeing in the presence of a colorless compound of the formula



if desired or required, together with a weakly cation-active, complex-forming agent.

In the above Formula I

R represents hydrogen or a low molecular alkyl radical  
A represents an aliphatic, aromatic, araliphatic, or cycloaliphatic radical

Z represents an anion-active group such, for example, as  
—SO<sub>3</sub>Y, —OSO<sub>3</sub>Y, —COOY, —SO<sub>2</sub>CH<sub>2</sub>CH<sub>2</sub>OSO<sub>3</sub>Y.  
(Y=hydrogen or a salt forming cation, preferably an alkali metal cation)

n represents an integer from 1 to 3

X represents halogen, preferably chlorine or the group



wherein R, A, Z and n have the meanings given above.

As compounds of the Formula I, there are preferably used compounds in which R represents a hydrogen atom, A represents an alkylene radical having 1-4 carbon atoms, a phenylene radical, a naphthalene radical or a phenylene or naphthalene radical substituted by one or several nitro groups, amino groups, low molecular alkyl- or alkoxy radicals, and/or halogen, and Z, n and X have the meanings given above.

The compounds of the present invention permit dyeing at temperatures of up to 130° C. without the addition of protective agents and without incurring the risk of damaging the fibers. By application of this high temperature, in many cases the yield and the levelness are rather improved.

Another advantage in the use of the assistants of the present invention is that dull shades on polyamide textiles are obtained, since in practice the luster of the dyed goods has always been objected to.

The assistants having the Formula I can be prepared, for example, by reacting amines of the formula



with cyanuric chloride preferably in an aqueous medium, at a reaction temperature ranging from 0 to 100° C., while neutralizing the hydrogen chloride liberated.

As neutralizing agents, there may be preferably used mineral acid-binding agents, for example, alkali metal hydroxides, carbonates or hydrogen carbonates, and alkaline earth metal hydroxides, carbonates or hydrogen carbonates.

As amines of the general formula



there may be used:

1-aminobenzene-2-sulfonic acid  
1-aminobenzene-3-sulfonic acid

- 1-aminobenzene-4-sulfonic acid
- 1-aminobenzene-2,4-disulfonic acid
- 1-aminobenzene-2,5-disulfonic acid
- 4-aminotoluene-2-sulfonic acid
- 5 1-aminobenzene-4-chloro-3-sulfonic acid
- β-amino-ethanol-sulfuric acid ester
- β-N-methylamino-ethanesulfonic acid
- 1-aminobenzene-3-carboxylic acid
- 1-aminobenzene-4-carboxylic acid
- 10 1-aminobenzene-3-β-hydroxyethylsulfone-sulfuric acid ester
- 1-aminobenzene-4-β-hydroxyethylsulfone-sulfuric acid ester
- β-sulfato-propionic acid-(p-amino-phenylamide)
- 15 β-sulfanilamido-monethyl sulfate
- β-(N-methyl-N-p-aminophenyl-sulfamide)-monethyl sulfate
- 2-amino-5-sulfobenzoic acid
- 1-aminocyclohexane-4-sulfonic acid
- 20 1-naphthylamino-3,6-disulfonic acid
- 2-aminonaphthalene-5-sulfonic acid

The 2,4,6-s-triazine-tri-aminobenzene-β-hydroxyethylsulfone sulfuric acid esters can also be prepared by reacting cyanuric chloride with aminobenzene-β-hydroxyethylsulfone in the melt or in a higher-boiling organic solvent, for example, xylene and subsequent esterification of the trihydroxy compound formed with concentrated sulfuric acid.

25 As complex-forming, weakly cation-active products which may be used, if required or desired, together with the compounds of the Formula I, there enter into consideration, for example, the addition products of alkylene oxide to alkylamines or polyalkylene polyamines, preferably the compounds obtained by the addition of 2-30 mols of ethylene oxide to 1 mol of an alkylamine having at least one alkyl radical with 8-18 carbon atoms or of a substituted alkylamine, for example, a compound of the

30 formula



- 35 in which R' stands for an alkyl radical having 8-18 carbon atoms, or 1 mol of a polyalkylene polyamine such as ethylene diamine, diethylene triamine or hexamethylene diamine; condensation products of melamine, formaldehyde and one compound obtained by the addition of 40 preferably 8-80 mols of ethylene oxide to 1 mol of triethanolamine, or the products obtained by acid condensation of formaldehyde and addition products of alkylene oxide, preferably of 8-50 mols of ethylene oxide to 1 mol of a mixture of a simple aromatic amine such, for example, as aniline and a phenol, and, if required or desired, a low molecular alkanolamine, especially triethanolamine. Furthermore, there may be used the quaternization products of the above-specified compounds, for example, those obtained by the reaction with dimethyl sulfate.
- 45 The ratio of the anion-active to the cation-active compound used if desired or required, can vary within wide limits. Thus, as has already been mentioned, the anion-active compounds encompassed by the Formula I may be used with good results alone. When mixtures of the mentioned anion-active and cation-active compounds are used, the ratio of the individual components may be adjusted to the prevailing circumstances of each individual case. The components can be used in equal amounts, but 50 it generally proved advantageous to use an excess of

anion-active compound. It is preferred to use a ratio of 3 parts by weight of anion-active compound to 1 part by weight of cation-active compound.

For stabilization, there may be added to the mixtures of anion-active and cation-active compounds, if desired or required, about 0.5-2% of a non-ionic surface-active compound, for example, the product obtained by the addition of 20-40 mols of ethylene oxide to 1 mol of an alkyl phenol having an alkyl radical with about 8-12 carbon atoms.

The dyeing conditions, such as the dyebath temperature, the pH of the dyebath, the proportion of dyestuff in the dyebath and the liquor ratio, may be varied as desired. Thus the dyebath is preferably heated to a temperature of at least 80 to 90° C.; mostly, the dyeing is carried out at the normal boiling point of the dyebath. Augmentation of the dyeing temperature to about 120-130° C. is possible, but is in most cases not necessary to obtain streakless dyeings with good depth of shade. The dyebath should have an acid pH. The pH value may range between about 3 and 6, preferably between 3 and 4.

In comparison with the quantity used of other known assistants, the small quantity of 0.5-3 percent by weight of the anion-active dyeing assistant or of the mixture of anion-active and cation-active substances according to the invention, which gives good results even with deep shades, is a considerable advantage. In many cases, a quantity of only 0.5-2 percent by weight, referred to the weight of the goods, will already be sufficient.

When using the compounds or mixtures according to the present invention, streakless, level dyeings on polyamide fibrous materials will be obtained. Changes of the depth of shade and of the shade itself do not occur or only in a practically insignificant degree. The drawbacks of the known processes are thereby obviated.

Furthermore, when using the products in the dyeing of polyamide fibers with acid wool dyestuffs, good wetting and rubbing fastnesses are obtained. Especially good results will in this case be obtained when using as anion-active compounds of the Formula I such as contain the group  $-\text{SO}_2-\text{CH}_2-\text{CH}_2-\text{OSO}_3\text{Y}$  (Y having the meaning given in Formula I) and rinsing the goods after dyeing for 1 to 20 minutes at temperatures in the range of 60 and 90° C. with an aqueous alkaline bath in the presence of a high molecular compound containing at least 3 hydroxyl groups. During this treatment in the alkaline medium, there form reactive vinylsulfone groups in the anion-active dyeing assistant which cause cross-linking with the added compounds containing hydroxy groups. This fastness-improving treatment can also be carried out by padding with alkalies and compounds containing hydroxyl groups the dyeings produced on polyamide fabrics in the presence of compounds of the Formula I containing the group



and then further treating the fabric as usual on the stenter at temperatures in the range of 90 and 180° C. for a period from 30 seconds to 10 minutes.

As alkalies for the aftertreatment, there may be used in particular alkali metal hydroxides, alkali metal carbonates and alkali metal bicarbonates, as well as alkali metal salts of organic acids which pass over into hydroxides or carbonates at elevated temperatures. There are mentioned by way of example: sodium hydroxide, potassium hydroxide, sodium carbonate, potassium carbonate, and the corresponding bicarbonates, sodium acetate, potassium acetate as well as the sodium or potassium salt of trichloroacetic acid.

The alkalies are generally used in amounts from about 0.3 to 10 percent by weight, preferably 0.3 to 5 percent

quantity should be so chosen as to give a pH of at least by weight, referred to the weight of the goods. The 8. If compounds are used, which pass into alkalies at elevated temperatures, for example, the sodium salt of trichloroacetic acid, one can work under neutral or weakly acid conditions.

As higher molecular compounds of synthetic origin, with alcoholic hydroxyl groups, there enter into consideration for example, polyvinyl alcohols having K-values from about 10 to 100 (according to Fickentscher, Cellulosechemie, tome 13, page 58 (1932)), polyvinyl alcohols which can be either fully hydrolyzed or partly hydrolyzed and have a residual acetyl content of 0-90% as well as polyvinyl acetals containing hydroxyl groups, i.e. partly acetalized polyvinyl alcohols, for example, acetalized with formaldehyde, acetaldehyde, benzaldehyde or other aliphatic or aromatic aldehydes, with an acetalization degree of 0-99% and K-values from 10 to 100. Furthermore, copolymers of monomeric vinyl compounds such as vinyl chloride, acrylic acid esters, methacrylic acid esters, acrylonitrile, styrene, etc. with vinyl esters such as vinyl formate, vinyl acetate, vinyl propionate, etc., into which hydroxyl groups have been introduced by partial hydrolysis. The proportion of vinyl ester groups in the mentioned copolymers can vary between 0.5 and 99%, the degree of hydrolyzation of the vinyl ester component can vary from about 10 to 100%. Furthermore, there are also suitable resins or partially hydrolyzed graft polymers of vinyl esters with polyethylene glycols, for example, those obtained according to the German specifications 1,081,229 and 1,094,457.

As hydroxyl-containing compounds of natural origin there may be used *inter alia* carbohydrates such as starches (wheat starch, rice starch, potato starch, etc.) tragacanth, tannine, locust bean flour as well as locust bean flours that are partially etherified with lower mono- or dihydric aliphatic alcohols having 1-4 carbon atoms, modified starch preparations for example, British rubber, sugar, and sugar alcohols, furthermore cellulose esterified with lower carboxylic acids or lower alcohols having 1-4 carbon atoms or etherified cellulose, for example, methyl cellulose, carboxymethyl cellulose, etc.

The following examples illustrate the invention, but they are not intended to limit it thereto:

#### Example 1

100 parts of a polyamide fabric consisting in warp and beam of endless filaments, normally dyeing with streaks only, are dyed in a closed dyeing apparatus for 1 hour at 100° C. with 2 parts of an acid wool dyestuff strongly responding to yarn irregularities and having the general formula



65

70

75

3 parts of acetic acid (30% strength)  
3 parts of the compound



1000 parts of water. After having brought the dyebath to the above temperature in the course of 40-50 minutes. After rinsing and drying, there is obtained a streakless, fast, grey dyeing.

An improved fastness can be obtained, when treating 15 the goods in the first rinsing bath with

2 parts of sodium trichloroacetate, or  
2 parts of sodium bicarbonate alone or together with  
2 parts of tannine for 20 minutes at 60-80° C.

Equally good results are obtained when carrying out the process with 2 parts of a sodium hydroxide solution (32.5%) at 20° C.

The described aftertreatment can be carried out by padding on a foulard and drying the dyed fabric on a stenter for 5 minutes at 140° C.

In each case, dull colored goods having a convenient handle are obtained.

#### Example 2

100 parts of the fabric described in Example 1 are dyed as described in Example 1 with a dyebath having the following composition:

3 parts of the acid wool dyestuff of the constitution



0.5 part of a condensation product of 1 mol of stearyl amine and 12 mols of ethylene oxide (30% strength),  
1.5 parts of 2,4,6-tri-(1-aminobenzene-4-sodium sulfonate)-s-triazine,  
3 parts of acetic acid (30% strength),  
1000 parts of water.

When dyeing at a temperature of 100° C., there is already obtained a fast, streakless blue dyeing. Dyeing temperatures of 130° can also be used with good results.

As cation-active compound there can be used instead of 0.5 part of the condensation product of 1 mol of stearylamine and 12 moles of ethylene oxide, with the same success 1 part of polyvinylpyrrolidone.

#### Example 3

100 parts of the polyamide fabric which can be dyed with streaks only and which is described in Example 1, are dyed with 2 parts of the complex chrome 2:1 dyestuff obtained from 2 molecules of the following compound:



50

2 parts of the reactive dyestuff of the constitution



65

3 parts of 2,4,6-tri-(1-aminobenzene-3-potassium sulfonate)-s-triazine,  
1 part of the condensation product from 12 mols of ethylene oxide and 1 mol of stearylamine (30%),  
70 2 parts of acetic acid (30% strength),  
1000 parts of water.

75

After rinsing and drying, there is obtained a streakfree fast yellow dyeing corresponding in depth of shade and shade to an untreated dyeing.



3,400,121

11

in which Y is hydrogen or an alkali metal cation and n is 2.

3. A symmetrical 2,4,6-triazine of the formula



12

in which Y is hydrogen or an alkali metal cation and n is 1 or 2.

References Cited

UNITED STATES PATENTS

2,742,466 4/1956 Randall et al. ----- 260—249.5

OTHER REFERENCES

Beilstein's Handbuch der Organischen Chemie, vol. 26,  
4th ed., p. 75, system No. 3889, Erstes Ergänzungswerk (1938).

JOHN D. RANDOLPH, *Primary Examiner.*